

# UNITED STATES PATENT OFFICE.

WILHELM HELMUTH SCHWEITZER, OF HEIDELBERG, GERMANY, ASSIGNOR TO  
SOCIETY TECHNOCHEMIA AKTIENGESELLSCHAFT, OF GLARUS, SWITZER-  
LAND.

## MIXED TEXTILE GOODS AND PROCESS OF MAKING SAME.

1,413,621.

Specification of Letters Patent. Patented Apr. 25, 1922.

No Drawing.

Application filed April 28, 1921. Serial No. 465,290.

To all whom it may concern:

Be it known that I, WILHELM HELMUTH SCHWEITZER, a citizen of the German Republic, and resident of Heidelberg, Germany, have invented a new and useful 5 Mixed Textile Goods and Process of Making Same, of which the following is a full, clear, and exact specification.

By mixing wool, hairs or other animal 10 fibres together with the known artificial cellulose fibres, the resulting mixed textile goods has an appearance of a simple mixture.

I have now found that by mixing an improved textile animal fibre obtained according 15 to my two U. S. Letters Patents No. 1,389,274 and No. 1,389,275 dated August 30, 1920, with the said known artificial cellulose fibres, there results a mixed textile 20 goods having the appearance of a goods made of only one kind of fibre, and showing in a wet state, a greater fastness than textile goods made only of artificial cellulose fibres.

The new mixed textile goods are substitutes of cellulosic artificial silks, which are 25 cheaper than the new animal textile products described in my U. S. Letters Patent No. 1389274 and No. 1389275 and show against water a sufficient fastness, when as 30 shown in the following example, the proportion of the new animal textile product is in the new mixed textile goods at least one half by weight of the artificial cellulose fibres.

### Example.

35 50 kilos tops (wool slivers) previously treated successively with 100 per cent of chloride of lime and soda lye (caustic soda) and subsequently soaped, as described in 40 the above cited specification, are mixed on the gill-box with 100 kilos of combed artificial cellulose fibre (artificial silk) of any degree of fineness and spun in the usual way.

The unitary lustrous appearance is not 45 changed after dyeing.

The proportion of the new animal textile product in the new mixed textile goods can obviously be more than  $\frac{1}{2}$  of the weight of the mixture. But there is obtained generally a practically sufficient fastness of the mixed textile goods against water, when the proportion is that given in the above example.

### What I claim is:

1. As a new article of manufacture the herein described mixed lustrous textile goods having the appearance of a goods made of only one kind of fibre, and being formed by a mixture of one of the known 60 artificial cellulose fibres and of one of the new animal textile products resulting from the successive treatment of an animal fibre with an oxidizing agent and an alkaline substance, the proportion of the new animal 65 textile product being at least  $\frac{1}{2}$  of the weight of the new mixed textile goods which shows thus a sufficient fastness against water. 55

2. As a new article of manufacture the herein described mixed lustrous textile 70 goods having the appearance of a goods made of only one kind of fibre, and being formed by a mixture of one of the known artificial cellulose fibres, and the new animal textile product resulting from the successive 75 treatment of wool with an oxidizing agent and an alkaline substance, the proportion of the said new animal textile product being at least  $\frac{1}{2}$  of the weight of the new mixed textile goods, which shows thus a sufficient 80 fastness against water.

In witness whereof I have hereunto signed my name this 30th day of March, 1921, in the presence of two subscribing witnesses.

WILHELM HELMUTH SCHWEITZER.

### Witnesses:

FRIDA KURZ,  
AMAND RITTER.